

June 30, 1959

A. ZLETZ ET AL

2,892,305

ROCKET PROPULSION METHOD

Filed Feb. 16, 1953



INVENTORS:  
Alex Zletz  
Don R. Carmody  
BY  
Michael Dufresne  
ATTORNEY

1

2,892,305

## ROCKET PROPULSION METHOD

Alex Zletz, Park Forest, and Don R. Carmody, Crete, Ill., assignors to Standard Oil Company, Chicago, Ill., a corporation of Indiana

Application February 16, 1953, Serial No. 336,902

14 Claims. (Cl. 60—35.4)

This invention relates to the generation of gas. More particularly, it relates to reaction propulsion by the hypergolic reaction of a liquid fuel and a liquid oxidizer. Still more particularly, the invention relates to a method of rocket propulsion by the hypergolic reaction of a fuel and a hydrogen peroxide oxidizer, which materials spontaneously react to generate gas at high pressure and high temperature.

Reaction propulsion is now being used for many aerial purposes. For many uses it is necessary to operate with a fuel system which is not dependent on atmospheric oxygen. This fuel system may consist of a single self-contained propellant or it may consist of a separate fuel and a separate oxidizer, i.e., a bipropellant system.

In the bipropellant system the fuel and the oxidizer are introduced separately and essentially simultaneously into the combustion chamber of the reaction motor. The products of oxidation from the reaction of the fuel and the oxidizer are discharged through an orifice at the exit end of the combustion chamber and thereby produce the driving force. Because of the possibilities of electrical and/or mechanical failure of the auxiliary methods of ignition such as a spark or a hot surface, it is preferred to use a self-igniting fuel system. A fuel which is self-igniting, i.e., spontaneously combustible when contacted with an oxidizer, is known as a hypergolic fuel.

Temperature has an important effect on the hypergolic activity of fuels. The temperature at the earth's surface may vary from a high of about +125° F. to a low of as much as —65° F.; in general temperatures below about —20° or —30° F. are exceptional. Thus surface-to-air missiles or rocket-driven aircraft should be capable of operation when the temperature of the fuel and the oxidizer at the moment of initial contact in the combustion chamber of the rocket motor is on the order of —20° F. Temperatures at high altitudes are frequently on the order of —65° F. and are known to approach —100° F. Thus an air-to-air missile should be able to operate satisfactorily when the temperature of the fuel and the oxidizer at the moment of initial contacting in the combustion chamber is on the order of —65° F.

The more common oxidizers are white fuming nitric acid, red fuming nitric acid and nitric acid-sulfuric acid mixtures. While these nitric acid oxidizers operate satisfactorily over a wide range of atmospheric temperatures they have important drawbacks. The nitric acid oxidizers are extremely corrosive; they have poor storage stability; they give off toxic gases; and special precautions must be taken by personnel who handle these oxidizers.

Concentrated aqueous hydrogen peroxide solutions have excellent storage stability and do not give off harmful gas. However, these aqueous hydrogen peroxide solutions such as 90% hydrogen peroxide have the disadvantage of comparatively high freezing points, e.g., 90%

5 hydrogen peroxide solution freezes at +12° F. The freezing point of 80% hydrogen peroxide is —9° F., but the activity of this solution toward the prior art fuels is markedly lower than the 90% H<sub>2</sub>O<sub>2</sub> solution. The 10 freezing point of aqueous hydrogen peroxide solutions can be depressed by dissolving therein inorganic salts, preferably ammonium nitrate. Thus a solution containing 40 weight percent of ammonium nitrate and in which the hydrogen peroxide-water portion contains 90 weight percent of H<sub>2</sub>O<sub>2</sub> has a freezing point of about —30° F. A so-called 80% H<sub>2</sub>O<sub>2</sub>—30% NH<sub>4</sub>NO<sub>3</sub> solution has a freezing point of below —70° F.

15 Concentrated aqueous hydrogen peroxide solutions have been used as monopropellants by catalytically decomposing the hydrogen peroxide, using such catalysts as potassium permanganate or copper oxide. Since the decomposition products contain free-oxygen the monopropellant system is inefficient. However, fuels which are hypergolic with nitric acid oxidizers may be much 20 less active or even inactive with concentrated H<sub>2</sub>O<sub>2</sub> solutions. Anhydrous hydrazine is usually considered to be the only fuel that is sufficiently hypergolic with concentrated H<sub>2</sub>O<sub>2</sub> solutions to be practical; however, hydrazine has the disability of a comparatively high freezing 25 point. Some fuels are operative with H<sub>2</sub>O<sub>2</sub> solutions in the presence of a H<sub>2</sub>O<sub>2</sub> decomposition catalyst.

30 An object of this invention is a method of generating gas by the hypergolic reaction of a fuel and a hydrogen peroxide oxidizer. Another object is a method of reaction propulsion by the hypergolic interaction of a fuel and a hydrogen peroxide oxidizer. Still another object is a method of reaction propulsion by the hypergolic interaction of a hydrogen peroxide oxidizer and a fuel which contains appreciable amounts of miscible hydrocarbons, particularly non-hypergolic liquid hydrocarbons. Another particular object is a method of rocket 35 propulsion by the hypergolic interaction of a defined organic phosphine and a defined hydrogen peroxide oxidizer when the temperature of the fuel and the oxidizer is above about —20° F. Other objects will become apparent in the course of the detailed description of the invention.

40 A method has been discovered for generating gas, which gas may be used as a substitute for compressed air for certain purposes or for driving the turbine of a jet engine or for rocket propulsion, which method comprises contacting

45 (1) A fuel consisting essentially of at least one member selected from the class consisting of  
(A) Monoaliphatic phosphines which contain not more than 16 carbon atoms,  
(B) Dialiphatic phosphines which contain not more than 20 carbon atoms and wherein each aliphatic radical contains not more than 12 carbon atoms, and  
(C) Trialiphatic phosphines which contain not more than 24 carbon atoms and wherein each aliphatic radical contains not more than 12 carbon atoms, and

50 (2) An oxidizer selected from the class consisting of  
(i) Aqueous hydrogen peroxide solutions which contain at least about 80 weight percent of H<sub>2</sub>O<sub>2</sub> and the remainder is essentially water, and  
(ii) Aqueous hydrogen peroxide-inorganic salt solutions wherein the hydrogen peroxide-water portion contains at least about 80 weight percent of H<sub>2</sub>O<sub>2</sub>.

55 Mono-octyl phosphines containing as much as 60 volume percent of miscible hydrocarbon are hypergolic with aqueous hydrogen peroxide solutions containing at least

about 90 weight percent of hydrogen peroxide when the fuel and the oxidizer are at a temperature of at least about +60° F.

Certain organic phosphines ignite spontaneously when contacted with "hydrogen peroxide oxidizers." The various phosphines do not have equal hypergolic activity with the same oxidizer. However, by proper selection of the phosphine, it is possible to obtain a hypergolic reaction with a tolerable ignition delay when the phosphine and the oxidizer are at a temperature of about -20° F. at the moment of initial contact in the gas generating chamber.

Certain monoaliphatic phosphines, dialiphatic phosphines, trialiphatic phosphines and mixtures thereof are useful for the purposes of this invention. These aliphatic phosphines have the generic empirical formula  $RR'R''P$  where P represents the element phosphorus, R represents an aliphatic radical and R' and R'' represent the same or different radicals selected from the class consisting of aliphatic and hydrogen. The term "aliphatic" as used herein is intended to include hydrocarbon radicals selected from the class consisting of paraffins, olefins and naphthenes. In the case of naphthenic radicals, the radical may be attached to the phosphorus either through a ring carbon atom or through a side chain carbon atom. It has been found that the highly branched aliphatic substituents have desirably lower freezing points than the straight chain or slightly branched substituents. It is preferred to use branched aliphatic substituents. The presence of unsaturated linkages in the aliphatic substituent improves the hypergolic activity. A particularly useful aliphatic phosphine contains not only a highly branched aliphatic radical, but also contains one or more unsaturated linkages.

It has been found that the hypergolic activity of the various aliphatic phosphines is dependent upon the number of aliphatic radicals, upon the total number of carbon atoms contained in the phosphine, and upon the number of carbon atoms contained in each of the aliphatic radicals. In order to obtain a fuel which is usable at low temperatures, it is necessary that the monoaliphatic phosphines contain not more than 16 carbon atoms. The phosphines which contain two aliphatic radicals, i.e., dialiphatic phosphines, must contain not more than 20 carbon atoms in the molecule and furthermore, each aliphatic radical must not contain more than 12 carbon atoms. Thus a dialiphatic phosphine which contains a 12 carbon atom side chain must not contain more than 8 carbon atoms in the second side chain. The completely substituted phosphines, i.e., trialiphatic phosphines, must not contain more than 24 carbon atoms in the molecule and furthermore, no aliphatic radical must contain more than 12 carbon atoms. Thus a trialiphatic phosphine which contains a 12 carbon atom side chain will contain only, for example, two hexyl or one octyl and one butyl radical as the other radicals.

When it is desired to initiate the combustion at low temperatures on the order of -20° F., it is preferred to use the following fuels: monoalkyl phosphines which contain not more than 8 carbon atoms; dialkyl phosphines which contain not more than 12 carbon atoms and wherein each alkyl radical contains not more than 8 carbon atoms; trialkyl phosphines containing not more than 12 carbon atoms total and not more than 8 carbon atoms in any alkyl radical. The preferred species for operation at starting temperatures of about -20° F. are the tributyl phosphines and mono-n-octyl phosphine.

A mixed fuel which is suitable for the generation of gas for reaction propulsion when the fuel and the oxidizer are at a temperature of at least about +60° F. can be made by mixing an alkyl phosphine which contains not more than 12 carbon atoms with a miscible hydrocarbon. An effective amount of phosphine must necessarily be present in the mixed fuel in order to obtain the hypergolic reaction. This amount will vary with both the type of hydrocarbon

and the species of phosphine. When using a mono-octyl phosphine and aromatic hydrocarbon mixture, as much as 60 volume percent of the mixed fuel may be aromatic hydrocarbons. In general petroleum hydrocarbon fractions 5 are suitable materials, for example, those fractions boiling between about 300° and 600° F. which correspond to the fuel requirement of military jet engines. Aromatic hydrocarbons which boil below about 600° F. are suitable hydrocarbons for this purpose. The hypergolic activity of the mixed fuel can be improved at temperatures below about +60° F. by using as the hydrocarbon component olefinic hydrocarbons such as thermally cracked naphthas and gas oils or turpentine. Conversely, at temperatures above about 60° F., a hypergolic 15 mixed fuel containing less than about 40 volume percent of mono-octyl phosphine is obtainable by the use of olefinic hydrocarbons.

The oxidizers of this invention are either concentrated aqueous hydrogen peroxide solutions or aqueous hydrogen peroxide solutions containing dissolved inorganic salts, for example, ammonium halides, sodium sulfate, sodium nitrate, etc.; the inorganic nitrates are preferred. The concentrated aqueous hydrogen peroxide solutions should contain at least about 80 weight percent of  $H_2O_2$ ; 25 the remainder of the solution is essentially water.

The hypergolic activity of the aqueous hydrogen peroxide solution is improved by increasing the concentration of the peroxide. Commercially available 90%  $H_2O_2$  solution is a preferred oxidizer. Still more concentrated 30 solutions are better when operation above the freezing point of the solution is desired.

Concentrated aqueous hydrogen peroxide solution as made commercially is virtually only  $H_2O_2$  and water. In order to improve storage stability small amounts of stabilizers 35 may be added to the solution, e.g., sodium stannate, tetrasodium pyrophosphate, adipic acid, tartaric acid; in general only trace amounts of stabilizers are added so that the solution consists essentially of hydrogen peroxide and water.

In order to depress the freezing point of aqueous hydrogen peroxide solutions soluble inorganic salts are dissolved therein, e.g., sodium nitrate, ammonium chloride and ammonium nitrate have been used. The preferred salt is ammonium nitrate. These salt-containing solutions are commonly designated in terms of the weight percent of salt in the total solution and the weight percent of hydrogen peroxide present in the aqueous portion of the solution, e.g., 90%  $H_2O_2$ —40%  $NH_4NO_3$  indicates that the total aqueous hydrogen peroxide-nitrate solution consists of 40 weight percent of ammonium nitrate and 60 weight percent of aqueous hydrogen peroxide composed of 90 weight percent of  $H_2O_2$  and the remainder essentially water. This particular solution has a freezing point of about -30° F. A temperature of -70° F. is attainable with an 80%  $H_2O_2$ —30%  $NH_4NO_3$  solution. It is preferred to operate in the absence of soluble inorganic salts because these salts have an adverse effect on the hypergolic activity of the fuels of this invention.

The aliphatic phosphines are in general clear, mobile, high-boiling liquids with an unpleasant odor. They are fairly stable when exposed to elevated temperatures in the absence of air, but are extremely susceptible to oxidation by air even at ambient temperatures. Thus they are quite stable when stored in sealed containers such as stoppered flasks and stainless steel drums.

Several methods are known for the preparation of the aliphatic phosphines, e.g., the method of W. C. Davies and W. J. Jones as described in J. Chem. Soc. (London), p. 33 (1929); also, that of W. C. Davies in J. Chem. Soc. (London), p. 1043 (1933). Both of these methods involve the Grignard reaction. However, it is preferred to use the method described in U. S. Patent 2,584,112 which involves the reaction of phosphine and an olefin.

The products from all of these methods of preparation contain minor amounts of impurities. These impurities

have a favorable effect on the freezing point of the aliphatic phosphines and appear to have no substantial adverse effect on hypergolic activity. It has also been found that the aliphatic phosphines which have been oxidized to a minor extent, e.g., 4 or 5%, are useful as hypergolic fuels. It is intended to include within the scope of the invention the use of aliphatic phosphines which contain minor amounts of impurities resulting from the preparation thereof and also those which contain minor amounts of oxidation products resulting from the oxidation of the aliphatic phosphine.

The aliphatic phosphines are particularly suitable fuels for rocket propulsion because of their low freezing points, high boiling points, and small increase in viscosity with decrease in temperature. In addition to their low freezing points they also have a considerable tendency to supercool, i.e., remain liquid at temperatures below the true freezing point. Most of these compounds do not form a crystalline mass when solid, but solidify in the form of a glass.

Several aliphatic phosphines were prepared by the methods of the literature. The method of Davies and Jones supra was used to prepare a high purity tri-n-butyl phosphine. The method of Davies supra was used to prepare a high purity tri-secondary butyl phosphine, and also trimethyl phosphine. The method of U.S. Patent 2,584,112 was used to react n-octene, 2-ethyl-1-hexene and a propylene tetramer with phosphine. In each case a mixture of substituted phosphines resulted and this mixture was carefully fractionated to produce cuts which were predominantly mono, di and tri-alkyl phosphines. The physical characteristics of some of the materials which were used in the tests to be described later are listed below:

| Phosphine                   | Specific Gravity (75° F.) | B.P.    |       | F.P., °F.          |
|-----------------------------|---------------------------|---------|-------|--------------------|
|                             |                           | ° F.    | mm.Hg |                    |
| Tri-n-butyl                 | 0.82                      | 295-307 | 50    | <-90               |
| Di (2-ethylhexyl)           | 0.8                       | 260-410 | 50    | <-90               |
| Mono (2-ethylhexyl)         | 0.83                      | 347-352 | 750   | <-100              |
| Mono (n-octyl)              | 0.82                      | 207-248 | 50    | +14                |
| Mono (dodecyl) <sup>1</sup> | 0.82                      | 140-150 | 0.5   | <sup>2</sup> <-100 |

<sup>1</sup> Propylene tetramer.

<sup>2</sup> Very viscous fluid.

The ignition characteristics of various fuels were studied using a "drop" test. This method utilizes a test tube, 1 in. x 4 in., containing about 0.5 ml. of oxidizer. The fuel to be tested was drawn into a hypodermic syringe. It was then ejected forceably against the oxidizer surface by depressing the syringe plunger. By this method amounts of fuel of as little as 0.01 ml. can be added. Low temperature tests were carried out by cooling the test tube and the oxidizer contained therein by means of a bath; a drying tube inserted into the top of the test tube excluded moisture. The fuel was cooled separately to the desired test temperature. By supercooling it was possible to carry out tests at temperatures below the freezing point of the fuel and/or the oxidizer.

The "ignition delay," which is the time elapsing between the addition of fuel to the oxidizer and visual ignition thereof, was determined visually as either (a) very short which corresponds to substantially instantaneous ignition, (b) short, which corresponds to substantially less than 1 second, and (c) more than 1 second, which time was determined by a stop watch.

The following tests illustrate the activity of some of the alkyl phosphines of this invention and hydrazine with hydrogen peroxide oxidizers.

#### Test I

Various phosphines were tested for hypergolic activity at a temperature of about +70° F. using 0.5 ml. of 90% H<sub>2</sub>O<sub>2</sub> as the oxidizer.

| Run No. | Fuel                             | Fuel Added, ml. | Ignition Delay            |
|---------|----------------------------------|-----------------|---------------------------|
| 5. 1    | Mono (n-octyl) <sup>b</sup>      | 0.04            | Very short.               |
| 2       | Mono (n-octyl)                   | 0.02            | Short.                    |
| 3       | Mono (2-ethylhexyl) <sup>c</sup> | 0.03            | Do.                       |
| 4       | Di (2-ethylhexyl)                | 0.05            | 1 sec.                    |
| 5       | Tri (2-ethylhexyl)               | 0.10            | No ignition. <sup>a</sup> |
| 6       | Mono (dodecyl) <sup>d</sup>      | 0.12            | Do.                       |
| 7       | Mono (dodecyl)                   | 0.20            | Short.                    |
| 8       | Tri (n-butyl)                    | 0.01            | Very short.               |
| 9       | Tri (sec-butyl)                  | 0.04            | Do.                       |

<sup>a</sup> Considerable effervescence.

<sup>b</sup> Prepared from 1-octene.

<sup>c</sup> Prepared from 2-ethylhexene.

<sup>d</sup> Prepared from propylene tetramer.

#### Test II

In this test several runs were made contacting various phosphines at about +70° F. using 80% H<sub>2</sub>O<sub>2</sub> solution as the oxidizer.

| Run No. | Fuel                | Fuel Added, ml. | Ignition Delay               |
|---------|---------------------|-----------------|------------------------------|
| 25. 10  | Mono (n-octyl)      | 0.06            | No ignition (effervescence). |
| 11      | do                  | 0.08            | Short.                       |
| 12      | Mono (2-ethylhexyl) | 0.06            | Do.                          |
| 13      | Tri (n-butyl)       | 0.06            | Do.                          |

#### Test III

In this test several runs were made using various phosphines at different temperatures with either 90% H<sub>2</sub>O<sub>2</sub> or 80% H<sub>2</sub>O<sub>2</sub> solutions as the oxidizer.

| Run No. | Fuel                | Fuel Added, ml. | H <sub>2</sub> O <sub>2</sub> Oxidizer, percent | Temp., °F. | Ignition Delay               |
|---------|---------------------|-----------------|-------------------------------------------------|------------|------------------------------|
| 40. 14  | Mono (n-octyl)      | 0.08            | 90                                              | 0          | 2 sec.                       |
| 15      | do                  | 0.12            | 90                                              | -20        | Short.                       |
| 16      | Mono (2-ethylhexyl) | 0.06            | 90                                              | 0          | 5 sec.                       |
| 17      | do                  | 0.14            | 90                                              | -20        | 4 sec.                       |
| 45. 18  | Tri (n-butyl)       | 0.08            | 90                                              | 0          | Very short.                  |
| 19      | do                  | 0.12            | 90                                              | -20        | Short.                       |
| 20      | Tri (sec-butyl)     | 0.10            | 90                                              | 0          | Do.                          |
| 21      | do                  | 0.14            | 90                                              | -20        | Do.                          |
| 22      | Mono (n-octyl)      | 0.08            | 80                                              | +14        | Do.                          |
| 23      | do                  | 0.08            | 80                                              | -20        | 2 sec.                       |
| 24      | Mono (2-ethylhexyl) | 0.06            | 80                                              | +14        | Do.                          |
| 50. 25  | do                  | 0.08            | 80                                              | -22        | 15 sec.                      |
| 26      | Tri (n-butyl)       | 0.12            | 80                                              | +14        | No ignition (effervescence). |

#### Test IV

For comparative purposes hydrazine was contacted at various temperatures with either 90% H<sub>2</sub>O<sub>2</sub> or 80% H<sub>2</sub>O<sub>2</sub> solutions as the oxidizer.

| Run No. | H <sub>2</sub> O <sub>2</sub> Oxidizer, percent | Fuel Added, ml. | Temp., °F. | Ignition Delay               |
|---------|-------------------------------------------------|-----------------|------------|------------------------------|
| 60. 27  | 90                                              | 0.05            | +70        | Very short.                  |
| 28      | 80                                              | 0.03            | +70        | Short.                       |
| 29      | 80                                              | 0.10            | +14        | No ignition (effervescence). |

#### Test V

In order to observe the effectiveness of phosphines with oxidizers consisting of aqueous hydrogen peroxide-ammonium nitrate solutions, a run was made using 0.5 ml. of a 90%-40% aqueous hydrogen peroxide-ammonium nitrate solutions as the oxidizer.

| Run, No. | Fuel            | Fuel Added, ml. | Oxidizer $H_2O_2-NH_4NO_3$ , percent | Temp., °F. | Ignition Delay, sec. |
|----------|-----------------|-----------------|--------------------------------------|------------|----------------------|
| 30.....  | Mono (n-octyl). | 0.02            | 90-40                                | +70        | 2                    |

Runs 2 and 30 show the adverse effect of dissolved ammonium nitrate on the ignition delay.

*Test VI*

The hypergolic activity of mixtures of phosphine and benzene was tested at about +70° F. using 0.5 ml. of 90%  $H_2O_2$  as the oxidizer.

| Run No. | Mixed Fuel              |                         |                       | Fuel Added, ml. | Ignition Delay            |
|---------|-------------------------|-------------------------|-----------------------|-----------------|---------------------------|
|         | Phosphine               | Phosphine, Vol. percent | Benzene, Vol. percent |                 |                           |
| 31..... | Mono(n-octyl).....      | 50                      | 50                    | 0.10            | No ignition. <sup>a</sup> |
| 32..... | do.....                 | 50                      | 50                    | 0.15            | Short.                    |
| 33..... | Mono(2-ethylhexyl)..... | 40                      | 60                    | 0.12            | No ignition. <sup>a</sup> |
| 34..... | do.....                 | 40                      | 60                    | 0.16            | 2 sec.                    |
| 35..... | Tri(n-butyl).....       | 90                      | 10                    | 0.20            | No ignition. <sup>a</sup> |
| 36..... | Tri(sec-butyl).....     | 90                      | 10                    | 0.20            | Do. <sup>a</sup>          |

<sup>a</sup> Effervescence.

It is obvious from the data presented above that this invention can be used to generate gas at high pressure. This gas can be used for operating machinery such as "compressed air hammers" or for aircraft catapults; another important use for this high pressure gas is in the starting of the turbines of jet-type engines. The invention is particularly useful for operations which require a compact power plant that is able to produce a large amount of energy over a very short period of time. Other examples of uses of this invention are: the rocket-assisted take-off or flight of aircraft; aerial missiles; boosters for surface vehicles.

The relative proportion of oxidizer-to-fuel used will depend upon the type of operation, the temperature of operation and the type of fuel and oxidizer being used. When using 90%  $H_2O_2$  solution as the oxidizer and tri-butyl phosphine as the fuel, between about 4.5 and 5.5 volumes of oxidizer are needed per volume of fuel.

By way of example this invention is applied to the propulsion of a ground-to-air missile. The annexed figure which forms a part of this specification shows schematically the bipropellant feed system and the motor of this missile. This same type of missile could be used as a ship-to-air missile. This missile is suitable for operations wherein the fuel and the oxidizer can be maintained at a temperature high enough to insure at least a short ignition delay, e.g., when using 90%  $H_2O_2$  as the oxidizer and tributyl phosphine as the fuel, a temperature of about -20° F.

In the drawing vessel 11 contains a quantity of gas at high pressure; this gas must be inert with respect to the oxidizer and the fuel; suitable gases are nitrogen and helium. Herein helium is used as the inert gas. Helium from vessel 11 is passed through line 12 and through valve 13 which regulates the flow of gas to maintain a constant pressure beyond valve 13. From valve 13 helium is passed through lines 14 and 16 into vessel 17 and simultaneously through line 18 into vessel 19.

Vessel 17 contains the oxidizer. Helium pressure forces the oxidizer out of vessel 17 through line 21 to valve 22. Valve 22 is a solenoid actuated throttling valve. Suitable electrical lines connect valve 22 to an electrical source and operating switch (not shown) at the control chamber at the launching site. The oxidizer is passed through line 23 and injector 24 into combustion chamber

26. Combustion chamber 26 is provided with an outlet nozzle 27.

Vessel 19 contains the fuel. Vessels 17 and 19 are constructed to withstand the high pressure imposed by the helium gas. The gas pressure forces fuel from vessel 19 through line 28 to solenoid actuated throttling valve 29. Valve 29 is similar in construction and in actuation to valve 22. The fuel is passed through line 31 and injector 32 into combustion chamber 26.

10 Valves 22 and 29 are of such a size and setting that a predetermined ratio of oxidizer-to-fuel is passed into combustion chamber 26. Injectors 24 and 32 are so arranged that the streams of oxidizer and fuel converge and contact each other forcibly, resulting in a very 15 thorough intermingling of the fuel and the oxidizer.

The missile is launched by activating the solenoids on valves 22 and 29. In this example 5.2 volumes of 90%  $H_2O_2$  solution per volume of phosphine is introduced into the combustion chamber. The oxidizer and the fuel react almost instantaneously upon contact in the combustion chamber; a large volume of very hot gas is produced in the combustion chamber, which gas escapes through orifice 27. The reaction from this expulsion of gas drives the missile toward its target.

25 Thus having described the invention, what is claimed is:  
1. A method of generating gas, which method comprises injecting separately and essentially simultaneously into the combustion chamber of a gas generator (1) a hypergolic fuel consisting essentially of a member selected from the class consisting of (i) monoalkyl phosphines containing not more than 8 carbon atoms, (ii) dialkyl phosphines containing not more than 12 carbon atoms and each alkyl radical contains not more than 8 carbon atoms and (iii) trialkyl phosphines containing not more than 12 carbon atoms and not more than 8 carbon atoms in an organic group, and (2) an oxidizer selected from the class consisting of (a) aqueous hydrogen peroxide solutions consisting of at least about 80 weight percent of  $H_2O_2$  and the remainder essentially water and (b) aqueous hydrogen peroxide-ammonium nitrate solutions wherein the hydrogen peroxide-water portion is the predominant component and consists of at least about 80 weight percent of  $H_2O_2$  and the remainder essentially water, in an amount and at a rate sufficient to initiate a hypergolic reaction with and to support combustion of the fuel.

2. The method of claim 1 wherein said fuel is tri-butylphosphine.

3. The method of claim 1 wherein said fuel is dioctylphosphine.

4. The method of claim 1 wherein said fuel is mono-dodecylphosphine.

5. The method of claim 1 wherein said fuel is mono-octylphosphine.

55 6. The method of claim 1 wherein said oxidizer consists of about 80 weight percent of  $H_2O_2$  and the remainder essentially water.

7. The method of claim 1 wherein said oxidizer consists of about 90 weight percent of  $H_2O_2$  and the remainder essentially water.

60 8. The method of claim 1 wherein said oxidizer consists of a solution of hydrogen peroxide, water and ammonium nitrate, wherein the nitrate content is about 30 weight percent and the hydrogen peroxide-water portion consists of about 80 weight percent of  $H_2O_2$  and the remainder essentially water.

9. The method of claim 1 wherein said oxidizer consists of a solution of hydrogen peroxide, water and ammonium nitrate, wherein the nitrate content is about 40 weight percent and the hydrogen peroxide-water portion consists of about 90 weight percent of  $H_2O_2$  and the remainder essentially water.

70 10. A method of generating gas, which method comprises injecting separately and essentially simultaneously into the combustion chamber of a gas generator (1) a

hypergolic mixed fuel consisting essentially of (I) a liquid miscible hydrocarbon and (II) monoocetyl phosphine and (2) an oxidizer selected from the class consisting of (a) aqueous hydrogen peroxide solutions consisting of at least about 80 weight percent of  $H_2O_2$  and the remainder essentially water, and (b) aqueous hydrogen peroxide-ammonium nitrate solutions wherein the hydrogen peroxide-water portion is the predominant component and consists of at least about 80 weight percent of  $H_2O_2$  and the remainder essentially water, in an amount and at a rate sufficient to initiate a hypergolic reaction with and to support combustion of the mixed fuel.

11. The method of claim 10 wherein said hydrocarbon is a liquid petroleum fraction boiling between about 300° and about 600° F.

12. The method of claim 10 wherein said hydrocarbon is a liquid aromatic hydrocarbon boiling below about 600° F.

13. The method of claim 10 wherein said hydrocarbon is a liquid olefin boiling below about 600° F.

14. The method of claim 12 wherein said hydrocarbon is benzene.

5

References Cited in the file of this patent

UNITED STATES PATENTS

|    |           |                |               |
|----|-----------|----------------|---------------|
| 10 | 53,695    | Somes          | Apr. 3, 1866  |
|    | 2,368,866 | Nygaard et al. | Feb. 6, 1945  |
|    | 2,573,471 | Malina et al.  | Oct. 30, 1951 |
|    | 2,584,112 | Brown          | Feb. 5, 1952  |

OTHER REFERENCES

- 15 Hackh's Chem. Dictionary, 3rd ed. (1944), pp. 30, 559.  
Jour. of Amer. Rocket Soc., No. 72, December 1947,  
pp. 17, 21, 26, 31-38.